

# United States Patent [19]

Przezdziecki

[11] 3,899,335

[45] Aug. 12, 1975

[54] **DIAZOTYPE ELEMENTS AND PROCESSES  
WITH CARBODIIMIDE DEHYDRATING  
AGENTS TO GENERATOR COUPLERS**

[75] Inventor: Wojciech Maria Przezdziecki,  
Pittsford, N.Y.

[73] Assignee: Eastman Kodak Company,  
Rochester, N.Y.

[22] Filed: Mar. 20, 1974

[21] Appl. No.: 452,895

[52] U.S. Cl..... 96/49; 96/75; 96/91 R

[51] Int. Cl.<sup>2</sup> ... G03C 1/58; G03C 1/60; G03C 5/34

[58] Field of Search..... 96/91 R, 75, 49

[56] **References Cited**

UNITED STATES PATENTS

|           |        |                       |          |
|-----------|--------|-----------------------|----------|
| 3,098,693 | 7/1963 | Sheehan.....          | 96/111 X |
| 3,100,704 | 8/1963 | Coles et al. ....     | 96/111   |
| 3,303,028 | 2/1967 | Aebi et al. ....      | 96/91 R  |
| 3,307,952 | 3/1967 | Aebi et al. ....      | 96/91 R  |
| 3,331,689 | 7/1967 | Sosnovsky et al. .... | 96/91 R  |
| 3,386,827 | 6/1968 | Aebi et al. ....      | 96/91 R  |
| 3,499,760 | 3/1970 | Amariti et al. ....   | 96/91 R  |

3,563,744 2/1971 Poot..... 96/91 R

FOREIGN PATENTS OR APPLICATIONS

983,665 2/1965 United Kingdom..... 96/91 R

Primary Examiner—Charles L. Bowers, Jr.

Attorney, Agent, or Firm—D. M. Schmidt

[57] **ABSTRACT**

A light-sensitive, heat-developable diazotype element comprising a light-sensitive diazonium salt, a solid carbodiimide dehydrating agent, and a solid coupler precursor in the form of an aminocarboxylic acid capable of producing a diazo coupler upon dehydration; and the method of using it to produce a visible dye image wherein the element is exposed to actinic radiation and then heated to the melting point of the dehydrating agent or coupler precursor to activate the dehydrating agent, and generate the diazo coupler which in turn reacts with undecomposed (unexposed) areas of the diazonium salt to yield an imagewise dye pattern. Optionally, an alkali precursor may be utilized in the element to accelerate dye formation.

8 Claims, No Drawings

**DIAZOTYPE ELEMENTS AND PROCESSES WITH  
CARBODIIMIDE DEHYDRATING AGENTS TO  
GENERATOR COUPLERS**

**BACKGROUND OF THE INVENTION**

**1. Field of the Invention**

This invention relates to novel light-sensitive, heat-developable diazotype elements, and in particular to the use of carbodiimides to generate diazo couplers in a layer comprising a diazo salt and a coupler precursor. The coupler is obtained by dehydration of the coupler precursor by the carbodiimide at an elevated temperature.

**2. Prior Art**

In U.S. Pat. No. 3,140,180, G. Fritz describes diazotype elements containing a thermolabile pyrrole compound having a carboxylic tertiary alkyl ester group which is capable of coupling after decarboxylation by heat.

U.S. Pat. No. 3,303,028 of C. M. Aebi et al. discloses thermodevelopable, light-sensitive diazotype compositions comprising a compound capable of being dehydrated to form a diazo coupling component in situ. The latent coupling component may be a  $\gamma$ -keto alcohol, a  $\beta$ - or  $\gamma$ -acid alcohol, a  $\gamma$ -lactone or mixtures thereof, which upon dehydration become compounds containing active methylene groups which are capable of entering color-forming or coupling reactions with diazonium salts. A preferred embodiment of the invention utilizes a cyanoguanidine compound as a dehydrating agent and as an alkali-precursor. In U.S. Pat. No. 3,307,952 to the same inventors provides for the formation of an unsaturated  $\beta, \beta'$ -unsaturated ketone diazo coupler by heating and dehydrating a  $\beta, \beta'$ -keto-alcohol.

U.S. Pat. No. 3,331,689 of G. Sosnovsky et al. describes a method which comprises heating to a decarboxylating temperature a normally stable acidic composition having in intimate contact a diazonium compound and an aromatic coupler precursor which contains a carboxylic group subject to decarboxylation when heated.

C. M. Aebi et al. in their U.S. Pat. No. 3,386,827 describe the use of thermolabile diazo coupler precursors such as 3-hydroxyglutaronitrile or  $\beta$ -hydroxy- $\beta$ -methyl glutaric acid. It is stated that: "It is believed that the coupling component is produced by splitting out water, an alcohol or a phenol formed by radical  $R_3O$  and hydrogen from which the carbon to which  $R_4$  is attached."

U.S. Pat. No. 3,499,760 of L. Amariti et al. discloses heat developable diazotype phototyping compositions in which a coupler containing an enolate structure is used. The system is able to couple under the influence of heat without requiring the use of alkaline solutions or vapors or alkaline generating compounds.

A. L. Poot et al. in U.S. Pat. No. 3,563,744 describe a thermodiazo copying material and process wherein a hydrazone compound decomposes upon heating to form a heterocyclic methylene base compound capable of coupling with a diazonium compound to form an azo dye image.

Most of the previous proposals for a heat developable diazo have achieved little or no commercial success, mainly because the coupler precursors and/or alkali precursors slowly decomposed, even at room temperature. Thus, decarboxylation of 2,4,6-trinitrobenzoic

acid can be carried out efficiently at 150°C. according to U.S. Pat. No. 3,331,689, but it is also likely to occur slowly at temperatures of 20° to 30°C. with resultant premature coupling. Also, the thermal dehydration of 5 certain carbonyl-containing coupler precursors as described, for example in U.S. Pat. No. 3,303,028, are relatively slowly generated unless an alkali precursor is utilized therewith. The alkali precursor, while speeding up the reaction, tends to decrease the storage stability 10 of the element.

**SUMMARY OF THE INVENTION**

The present discovery concerns improved photosensitive and thermally-developable diazotype elements 15 which process rapidly and exhibit better storage stability than those of the prior art.

This invention relates to methods and compositions of matter for generating azo dye images from light-sensitive, heat-developable diazotype compositions 20 comprising a light-sensitive diazonium compound, a normally solid carbodiimide dehydrating agent, and a normally solid diazo coupler precursor convertible by dehydration in reactive contact with the carbodiimide into a diazo coupler capable of reacting with said diazonium compound to form an azo dye. Preferably the coupler precursor is an aminocarboxylic acid that forms a heterocycle containing a reactive methylene radical when heated with said carbodiimide.

By the term reactive contact it is meant that the dehydrating agent and coupler precursor are contacted either in a liquid or with one of them in liquid form to produce the reaction conditions which bring about dehydration of the coupler precursor by the dehydrating agent. This latter reaction will not occur if the dehydrating agent and coupler precursor are in contact as 35 solids.

The dehydrating agent, when brought into reactive contact with the coupler precursor by melting of one of 40 these two components or an inert normally solid "solvent" reacts with the coupler precursor to free the coupler for a conventional dye-forming reaction with the diazo salt.

**SPECIFIC EMBODIMENTS OF THE INVENTION**

45 Three essential compounds are involved in the present invention and each of these components is a normally solid compound with a melting point of at least about 80°C., and preferably above about 100°C., in order to obtain the full benefits of the invention by 50 avoiding premature activation of the carbodiimide dehydrating component which converts the coupler precursor into the actual coupling agent. These components are:

- 55 1. the diazo salt;  
2. a carbodiimide dehydrating agent; and  
3. a coupler precursor which becomes a coupler upon dehydration.

Activation of the dehydrating agent occurs upon the 60 melting of the carbodiimide or any substance in contact with it, for example, the coupler precursor or an inert normally solid material which acts as a solvent, to bring the dehydrating agent and the coupler precursor into reactive contact.

Suitable light-sensitive diazonium compounds are 65 well known in the art as exemplified in the aforementioned prior art patents, especially in the disclosure of U.S. Pats. Nos. 3,303,028 and 3,761,263 which are in-

corporated herein by reference. Mixtures of such substances may also be employed. The preferred diazo salts include

|                                                 |               |              |
|-------------------------------------------------|---------------|--------------|
| parts include                                   |               |              |
| 1-diazo-4-(dimethylamino)benzene                |               | tetrafluoro- |
| boroborate                                      |               |              |
| 1-diazo-4-(cyclohexylamino)benzene              | phosphate     |              |
| 1-diazo-4-(diethylamino)benzene                 | chlorozincate |              |
| 1-diazo-4-(dehydroxyethylamino)-3-methylbenzene |               |              |
| sulfate                                         |               |              |
| 1-diazo-4-dimethylamino-3-methylbenzene         | chloros-      |              |
| tannate                                         |               |              |
| 1-diazo-4-(dimethylamino)-3-ethoxybenzene       | tetra-        |              |
| fluoroborate                                    |               |              |
| 1-diazo-4-(diethylamino)-3-chlorobenzene        |               |              |
| 1-diazo-2-carboxy-4-(diethylamino)benzene       | phos-         |              |
| phate                                           |               |              |

one of their amino hydrogens substituted with one of a wide variety of organic radicals including aliphatic (e.g., N-thiocarbalkoxy), cycloaliphatic (e.g., N-thiocarbamoylmorpholine), heterocyclic (e.g., N-2-5 benzothiazolyl), and aromatic (e.g., N-2-pyridyl) groups which may contain sulfur, oxygen, and nitrogen atoms. Such glycines may be defined as N-organic substituted glycines capable of dehydration and which upon dehydration yield compounds having a heterocyclic ring containing both a nitrogen and an active methylene radical capable of coupling to a diazonium compound. Very good results are obtainable with hippuric 10 acid and N-2-pyridylglycine.

Examples of compounds capable of dehydration to yield a heterocyclic ring containing an active methylene group capable of coupling with a diazo salt are:



1-diazo-4-morpholinobenzene tetrafluoroborate  
 1-diazo-4-morpholino-3-methoxybenzene tetrafluoroborate  
 1-diazo-4-morpholino-2-ethoxy-5-methoxybenzene chlorozincate  
 1-diazo-4-morpholino-2,5-dibutoxybenzene sulfate  
 1-diazo-2,5-diethoxy-4-benzoylaminobenzene phosphate

as well as those employed in the examples hereinabove. In some cases, this choice will be based upon one or more of such factors as the hue of the dye image, its brightness and resistance to fading as well as the cost of the diazo compound.

A more detailed description of useful diazonium salts and couplers is contained in U.S. Pat. No. 3,761,263 to Fleming et al. issued Sept. 25, 1973 which is incorporated herein by reference.

A variety of normally solid coupler precursors may be utilized as long as they are capable of being dehydrated, preferably rapidly, by the carbodiimide when brought into reactive contact therewith by melting of the carbodiimide, the coupler precursor or a normally solid "solvent" (as described hereinafter), to yield diazo coupling compounds. The coupler generated should desirably be substantially colorless and should, of course, be capable of coupling with the contiguous diazo salt, preferably in a rapid manner. As will be described below, coupling can be accelerated by rendering the reaction medium alkaline. Aminocarboxylic acids in general are suitable, especially glycines having

40 A number of carbodiimides may be utilized as chemical dehydrating agents as long as they exhibit good layer stability, i.e. substantially no dehydrating ability at room temperature. Also, they should preferably form substantially colorless products in their dehydrating action. A preferred class of carbodiimides are those having the formula:



wherein R<sup>1</sup> and R<sup>2</sup> may each individually represent substituted and unsubstituted organic radicals which include alkyl (e.g. methyl, ethyl, etc.), cycloalkyl (e.g. cyclohexyl), aralkyl, aryl and amine radicals and R<sup>2</sup> may also be a hydrogen atom. Among the many compounds suitable for the purposes described herein are:

55 DA-dehydrating agent  
 DA-1 dinaphthylcarbodiimide  
 DA-2 dicyclohexylcarbodiimide  
 DA-3 N-phenyl-N'-cyclohexylcarbodiimide  
 DA-4 di-p-dimethylaminophenylcarbodiimide  
 DA-5 N-tert-Butyl-N'-(triphenylmethyl)-carbodiimide  
 60 DA-6 1-Ethyl-3-(3-dimethylaminopropyl)-carbodiimide  
 hydrochloride

In applying the aforesaid components to various substrates of an absorbent nature (e.g., paper or cloth), it is often sufficient to merely dissolve the solid substances in a solvent, such as a conventional volatile organic solvent or mixtures thereof, that is subsequently evaporated to deposit the solute in and on the sub-

strates. When an impermeable substrate (e.g., a metal or polymeric sheet, polyethylene coated paper, etc.) is to be coated, the use of a vehicle or carrier which comprises a film-forming material is usually necessary. Techniques for accomplishing such coating are well known in the art. Among the many suitable conventional film-forming materials or binders suitable for this purpose are such resins as cellulose esters, acrylates, methacrylates, as well as polyvinyl alcohol, polyvinyl chloride, polyvinyl acetate, polyvinyl butyral, etc. Conventional diazo binders and supports, in addition to the foregoing, are well known in the art and further discussion of such materials here would serve no useful purpose.

Drying the treated substrate in unheated or gently heated circulating air may be necessary with a low melting component present in instances where the carbodiimide dehydrating agent is in contact with the coupler precursor, in order to avoid activating the coupler prematurely. However, premature activation can be

occurs. Third, the novel system is not sensitive to ambient humidity conditions until the fusion of one of the substances present occurs due to the nature of the mechanism of the conversion of the precursor into an active coupling agent by heating. Fourth, some carbodiimides, although excellent dehydrating agents at their melting point or in solution, have excellent solid state stability even in the presence of water.

It is also contemplated that conventional additives other than the binders may be employed provided that they do not interfere with the aforementioned reactions. These may be exemplified by stabilizers, extenders and thickeners to assist in coating operations.

These and additional objects and advantages of my invention will be evidenced by the following examples which are intended to be illustrative rather than limitations on the scope of the claims.

The following examples serve to illustrate particular embodiments of the present invention.

#### EXAMPLE 1



avoided by keeping these two components apart by separately depositing them on the substrate with a resin film between them or by depositing one of these components on the substrate and the other on a separate "developing sheet" that is placed on the substrate coating only shortly before dye image formation is desired.

For the formation of an image on a substrate coated or impregnated with a light-sensitive, heat-developable diazonium compound either alone or in combination with either the coupler precursor or the dehydrating carbodiimide, a latent image is formed by conventional exposure of the substrate through a photographic positive or other image pattern to actinic radiation, such as visible (if a suitable sensitizer is used) or ultraviolet light, arc lamps, etc. Next, the latent image is developed by heating the treated substrate while all three of the reactive substances are in intimate contact with one another (e.g., by laying a developing sheet onto a coating of diazo salt) to a suitable temperature to convert the precursor into a coupler by dehydration and to couple the coupler with undecomposed diazo compound in the unexposed areas to form a visible image colored by the resulting dye in such areas. Temperatures suitable for such dehydration and coupling will vary for different specific reactive components, and they may be easily determined by routine experimentation. As a guide, temperatures of the order of 110° to 130°C. have given excellent results with a number of the compositions described above and in the examples below.

The coupler-generating system of the instant invention provides important advantages. First, there is improved stability, since the coupler is not formed prematurely. The coupling agent is formed or released only when the melting point of one of the solid components is reached in the composition or coating. Second, activation of the active components of these compositions results in extremely rapid development of the dye image, even though the system is inert until such melting

Filter paper is imbibed with a solution of 0.1-g hippuric acid and 0.1-g 2,5-diethoxy-4-morpholinobenzene diazonium tetrafluoroborate in 5 ccs of a mixture of equal volumes of 2-Butanone and methanol. Since the above diagrammed dehydrating reaction occurs at a somewhat elevated room temperature using the dicyclohexylcarbodiimide, a second sheet of filter paper is imbibed with a solution of 0.1-g dicyclohexylcarbodiimide in 5 ccs of 2-butanone to produce a "developing sheet"; then both sheets are dried.

The first sheet is exposed for 7 sec. to ultraviolet light through a positive in the Kalcard 200 Exposer after which it was passed, in contact with the developing sheet, through heated rollers set at 110°C. Coupling of the nondestroyed (unexposed) diazo occurs rapidly to form red colored areas.

#### EXAMPLE II

1. A polyethylene terephthalate film base is coated with:

50 A 10% by weight solution of cellulose acetate butyrate in a solvent comprising 6 parts by volume acetone, 2 parts by volume methanol, and 1 part by volume methoxy ethyl acetate

|                                                              |         |
|--------------------------------------------------------------|---------|
| Hippuric Acid                                                | 10.0 g. |
| 2,5-Diethoxy-4-Morpholinobenzene diazonium tetrafluoroborate | 0.18 g. |
| To a wet thickness of about 4 mils                           | 0.10 g. |

60 2. A developing sheet is prepared by coating a paper support with:

A 10% by weight solution of cellulose acetate butyrate in solvent as in (1) above

|                                    |         |
|------------------------------------|---------|
| Dicyclohexylcarbodiimide           | 10.0 g. |
| To a wet thickness of about 4 mils | 0.21 g. |

After gently drying the coatings at a temperature of about 40°C for about 5 minutes, the coated film (1) is exposed to ultraviolet light for 30 sec. through a positive in the Kalcard 200 Exposer and then passed in contact with the developing sheet (2) containing the dehydrating agent through heated rolls set at 110°C. The undecomposed diazo couples with the coupler formed by dehydration of the hippuric acid, giving a dark red image.

## EXAMPLE III



The following coatings are prepared:

|         |                                                                                                  |         |
|---------|--------------------------------------------------------------------------------------------------|---------|
| Sheet 1 | N-2-pyridylglycine                                                                               | 0.23 g. |
|         | A 10% by weight solution of cellulose acetate butyrate in 80/20 weight ratio of acetone/methanol | 30.0 g. |

The above composition is coated at 4 mil wet thickness on subbed polyethylene terephthalate film.

|         |                                                      |         |
|---------|------------------------------------------------------|---------|
| Sheet 2 | Dinaphthylcarbodiimide                               | 0.55 g. |
|         | p-(Diethylamino) benzene diazonium tetrafluoroborate | 0.28 g. |

A 10% by weight solution of cellulose acetate butyrate in 80/20 weight ratio of acetone/methanol

This formulation is coated at 4 mil wet thickness on subbed poly(ethylene terephthalate). Subsequent to drying the coatings, Sheet 2 is imagewise exposed for 2 seconds to ultraviolet light using an IBM Micro Copier Model IID and then passed through rollers at 110°C. in contact with Sheet 1. A stable, reddish positive image is obtained, indicating formation of a coupler by dehydration. The color of the image is intensified by fuming with moist ammonia after the aforesaid heat treatment.

## EXAMPLE IV

Example III is repeated except that N-2-pyridylglycine is replaced in Sheet 1 with 0.29 g. of hippuric acid as the coupler precursor. A yellow image is obtained.

## EXAMPLE V

Example III is again repeated with dinaphthylcarbodiimide replaced in Sheet 2 with 0.56 g. of I (below) as an aminocarbodiimide dehydrating agent of the following structural formula:



A reddish-blue positive image is produced by processing as in Example III.

## EXAMPLE VI

A red image is obtained when another specimen of Sheet 2 of Example V is used with another Sheet 1 of Example IV.

## EXAMPLE VII

The following single sheet of three layer material is prepared.

Layer 3 as Sheet 2 of Example V  
Layer 2 5% Vistanex MM L-140\* (polyisobutylene in ligroin)

Layer 1 as Sheet 1 of Example III

\*A product of the Enjay Chemical Company.

The material is exposed for 4 seconds using an IBM Micro Copier Model IID and then processed on a heated block at 130°C. for 15 seconds. A stable, brown positive image is obtained.

While the invention has been described in detail with particular reference to preferred embodiments thereof, it will be understood that variations and modifications can be effected within the spirit and scope of the invention.

I claim:

1. A method of forming an azo dye image comprising the step of:

1. imagewise exposing to actinic radiation a supported layer comprising
  - a light-sensitive diazonium compound; and
  - at least one compound selected from at least one but not both of
    - i. a solid carbodiimide dehydrating agent having the formula



wherein  $R^1$  is an organic radical of the group consisting of alkyl, cycloalkyl, aralkyl, and aryl groups and amino derivatives thereof, and  $R^2$  is of the group consisting of hydrogen and said organic radicals, and

- ii. an N-organic substituted glycine convertible by dehydration, when placed in reactive contact with carbodiimide, into a heterocyclic active methylene coupler reactive with said diazonium compound to form an azo dye; and
2. heating said imagewise exposed layer while in contact with a layer comprising the other of (i) and (ii) to a temperature sufficient to cause said acid and said carbodiimide dehydrating agent to come into reactive contact thereby initiating formation of said coupler by dehydration and production of said azo dye image by reaction of said coupler with unexposed portions of said diazonium compound.
2. A method according to claim 1 wherein said glycine is selected from the group consisting of N-dithio-carbalkoxyglycines and N-thiocarbalkoxyglycines.

3. A method according to claim 1 wherein said carbodiimide is selected from the group consisting of dinaphthylcarbodiimide, dicyclohexylcarbodiimide, N-phenyl-N'-cyclohexylcarbodiimide, di-p-dimethylaminophenylcarbodiimide, N-tert-butyl-N'-(triphenylmethyl)-carbodiimide and 1-ethyl-3(3-dimethylaminopropyl)-carbodiimide hydrochloride.

4. A light-sensitive heat-developable diazotype imaging element comprising,

a. a layer comprised of a normally solid carbodiimide dehydrating agent having the formula



wherein  $R^1$  is an organic radical of the group consisting of alkyl, cycloalkyl, aralkyl and aryl groups and amino derivatives thereof, and  $R^2$  is of the group consisting of hydrogen and said organic radicals, and

b. a layer comprised of a an N-organic substituted glycine convertible by dehydration, when in reactive contact with said carbodiimide, into a coupler having a heterocyclic ring containing both a nitrogen atom and a coupling-reactive methylene radical, capable of coupling with a diazonium compound, wherein (a) and (a') are separate layers, one of said layers (a) and (b) further including a light-sensitive diazonium compound.

5. An element according to claim 4 wherein said glycine is selected from the group consisting of N-dithio-carbalkoxyglycines and N-thiocarbalkoxygly-

cines.

6. An element according to claim 4 wherein said carbodiimide is selected from the group consisting of dinaphthylcarbodiimide, dicyclohexylcarbodiimide, N-phenyl-N'-cyclohexylcarbodiimide, di-p-dimethylaminophenylcarbodiimide, N-tert-butyl-N'-(triphenylmethyl)-carbodiimide and 1-ethyl-3(3-dimethylaminopropyl)-carbodiimide hydrochloride.

7. A light-sensitive heat-developable diazotype composition for use with a coupler precursor capable of forming a coupler upon dehydration; the composition comprising, an admixture of a light-sensitive diazonium compound, and a normally solid carbodiimide dehydrating agent having the formula



wherein  $R^1$  is an organic radical of the group consisting of alkyl, cycloalkyl, aralkyl and aryl groups and amino derivatives thereof, and  $R^2$  is of the group consisting of hydrogen and said organic radicals.

8. A composition according to claim 7 wherein said carbodiimide is selected from the group consisting of dinaphthylcarbodiimide, dicyclohexylcarbodiimide, N-phenyl-N'-cyclohexylcarbodiimide, di-p-dimethylaminophenylcarbodiimide, N-tert-butyl-N'-(triphenylmethyl)-carbodiimide and 1-ethyl-3(3-dimethylaminopropyl)-carbodiimide hydrochloride.

\* \* \* \* \*

30

35

40

45

50

55

60

65

UNITED STATES PATENT AND TRADEMARK OFFICE  
CERTIFICATE OF CORRECTION

PATENT NO. : 3,899,335  
DATED : August 12, 1975  
INVENTOR(S) : W.J. Przedziecki

It is certified that error appears in the above-identified patent and that said Letters Patent are hereby corrected as shown below:

Column 9, line 22, "coupling reactive" should read  
--coupling-reactive--; line 24, "(a')" should read --(b)--.

Signed and Sealed this  
thirteenth Day of April 1976

[SEAL]

Attest:

**RUTH C. MASON**  
Attesting Officer

**C. MARSHALL DANN**  
Commissioner of Patents and Trademarks